

Sept. 2, 1952

O. W. FROST ET AL

2,608,911

CONCRETE FORM LINING MATERIAL

Filed May 1, 1946



INVENTORS  
Orcutt W. Frost &  
James H. Conover

*Fig. 1  
Orcutt W. Frost &  
James H. Conover  
Fig. 2  
Orcutt W. Frost &  
James H. Conover*

Patented Sept. 2, 1952

2,608,911

# UNITED STATES PATENT OFFICE

2,608,911

## CONCRETE FORM LINING MATERIAL

Orcutt W. Frost, Highland Park, and James H. Conover, Chicago, Ill., assignors to United States Gypsum Company, Chicago, Ill., a corporation of Illinois

Application May 1, 1946, Serial No. 666,513

13 Claims. (Cl. 92—40)

**1** The present invention concerns an improved material for lining forms such as are used in concrete construction. It is, usually, provided in the form of sheets of fibrous board from  $\frac{1}{2}$  inch in thickness, and upward, provided with a suitably absorbent surface.

It is essential that a material of this kind have the ability to absorb water from the freshly poured concrete surface and yet not to stick to it as the concrete hardens. The lining, in absorbing water from the surface, serves two purposes. It causes the surface to be harder, and also tends to reduce surface voids in the concrete by breaking any air bubbles and allowing the concrete to form a smooth surface against the lining. The lining must not stick to the hardened concrete when it is removed after setting, so that a clean surface is obtained.

Several types of form lining material purporting to serve this purpose are on the market at the present time. One consists of a fibrous sheet similar to cardboard, approximately  $\frac{1}{8}$ " thick and unsized so as to give it absorptive properties, having a large mesh cloth material, similar to cheesecloth, laminated to it to prevent sticking and surface voids. The other type consists of a fiber insulation board with a reduced amount of sizing to give absorptive properties, having the surface treated with an anti-sticking agent such as tannic acid.

Both types of material have the disadvantages of becoming soaked throughout and unusable if exposed to water before application. Care must be taken that they are not rained on before using. All packages and uncovered piles must, therefore, be protected on the job.

When used as a lining, these materials become soft and flimsy, due to absorbed water and any irregularities in the form material, such as that of rough wood, leaves a print on the hardened concrete. This makes it necessary to use high grade forming material.

It is one of the objects of the present invention to provide a lining material of relatively rigid form, which has a suitably water-absorbent surface that is of such nature that the set concrete or cement will not adhere thereto, therefore, permitting clean separation of the form from the resulting concrete or cement structure.

A further object of the present invention is to provide a process for the production of such a concrete-form lining material.

The invention is illustrated by two figures, of which Fig. 1 is a purely diagrammatic representation,

**2** in the merest outline, of a process of forming a fiber board, showing means for applying the coating or modifying composition of the present invention; and

**5** Fig. 2 is a cross section through one of the treated boards, shown in about twice actual size.

The product of the present invention is made of  $\frac{1}{2}$  inch insulation board, but is unsized and absorbent only to a depth of approximately  $\frac{3}{2}$  inch on one surface. The remainder of the board is well sized and consequently remains firm and stiff when used as a lining, so that rough wood may be used in making the forms. Also, in piles or packages, if only the sized water resistant surface is exposed, there is much less danger from exposure to water. Also in production of the fiber boards known to the art the degree of sizing must be carefully controlled to give the desired absorbency. A board with rapid absorbency is not suitable, as it draws the water too rapidly from the surface of the concrete. Such control of the degree of sizing is extremely difficult.

**25** The fiber insulation board of the present invention is made by the method known to the art as wet felting. The fibrous pulp is suspended in water to a consistency of usually about 1%, and rosin size and alum are added to give water resistance to the dry board. Waxes may also be used for sizing. The fibers are then deposited on a wire screen either by gravity or by suction, by allowing the water to be drawn away through the deposited fibrous mass. The wet felted mass is then pressed by rollers or the like, usually between wool felts or wire screens, to eliminate all the water possible and produce a compacted felted board which when dried will be approximately  $\frac{1}{2}$ " thick.

**30** After all possible water has been pressed out and before the wet mat is dried, a material is applied to the top surface in an amount that on penetrating the wet mat will be sufficient to neutralize the effect of the size to a depth that will give the desired degree of absorption on the dry board. This depth is generally approximately  $\frac{3}{2}$  inch. When the mat is dry, this, and only this, portion of the mat is absorptive, while the remainder will be well sized and water resistant.

**35** We have discovered that an aldehyde, such as formaldehydes or furfural when incorporated with the surface of the lining will act as an anti-sticking agent. We have further discovered that this type of material may be added as one of the ingredients of the above wet mat coating and still be effective after it is dried.

In one simple and economic operation, in addition to those of the regular process of insulation board manufacture, this coating material is applied to the wet mat and the resultant product is a new and improved form lining material.

The coating material is composed of a caustic material such as sodium hydroxide which acts to neutralize the size and an aldehyde, such for example as furfural, to act as an anti-sticking agent.

In order to prevent a reaction between the caustic and furfural, cold water must be used in preparing the coating and when using a caustic material such as sodium hydroxide, the ratio of caustic to furfural should not exceed one to 15 five.

The following is an example of a suitable coating composition:

|          | Parts |
|----------|-------|
| Water    | 300   |
| Furfural | 100   |
| NaOH     | 20    |

The caustic is dissolved in the cold water and the furfural is added with sufficient agitation until it becomes emulsified in the solution, after which the resulting emulsion may be applied to the mat surface.

In order to form a more stable emulsion, an emulsifying or wetting agent may be used. There are a large number of these now known and available; but it is preferable to employ one that is not affected by alkalies. This wetting agent will not only act as an emulsifying agent but also makes it possible to reduce the amount of caustic and consequently the furfural, thus producing a cheaper coating which will still give the desired water absorption properties. As an example one may use:

|               | Parts |
|---------------|-------|
| Water         | 300   |
| Furfural      | 50    |
| NaOH          | 12    |
| Wetting agent | 8     |

The wetting agent cannot be completely substituted for the caustic to give absorptive properties to the lining surface because the resultant mat will not meet the government specifications for form lining absorption. The specifications require that a lining surface of 16 square inches absorb between 6 to 16 grams of saturated lime water during the first 15 minutes, 15 to 26 grams in 60 minutes, and 18 to 29 grams in 120 minutes. If a wetting agent alone is used, almost all of the absorption is obtained in the first few minutes so that for 15 minutes the results are on the high side and practically no water is absorbed thereafter, at least not enough to meet the specifications. When caustic alone or a combination of caustic and the wetting agent is used, the caustic in the dried board dissolves in the absorbed water and tends to continue to neutralize the size so that the absorption is extended over a longer period and may be regulated to meet government specifications.

One of the wetting agents which we have found to be particularly well suited is a sulfonated hydrocarbon.

The method of application of the modifying material is substantially as follows (referring 70 to Fig. 1): A suitably sized cellulosic fiber furnish flows from stock-chest 3 through control-valve 4 into the Oliver type of board-former 5 upon the perforated or screen-covered drum 6 of which the board 7 is initially formed. The 75

freshly formed board then passes over the usual supporting belt 8 which travels on supporting rolls 9, being kept under suitable tension by passing over rollers 10 and 11. The belt is water-permeable, usually being made of some sort of felt, so that it may absorb the water from the board. The extraction of water from the freshly formed board is further aided by the use of the usual pressroll, such as roll 12. Usually, after 10 passing such a roll, there remains about 50% to 70% of water in the board. After passing this roll the composition of the present invention is applied to the board, as, for example, through a hopper 13 into which the composition is fed from a source of supply, as the storage tank 14, the flow being controlled by a valve 15 in pipe 16. The material will thus form a pool directly ahead of the spreading roll 17, which applies it evenly to the surface of the wet board. Thereafter the board may be cut by means of a traveling knife 18 and the lengths thus severed may pass onto an accelerated section of a conveyor 19 and thence, through the intermediate tipple 20, into a multi-deck drier 21 in which the boards are dried, being discharged from the latter through tipple 22 to be received on table 23. During the drying the sodium hydroxide contained in the coating composition will combine with the sizing material to form a sort of soap, whereby the sizing effect is destroyed, thus making the outer portions of the board much more receptive to moisture. At the same time the aldehyde will become deposited upon the fibers in that portion of the board where the applied composition has penetrated, which, as already pointed out, is about  $\frac{3}{4}$  of an inch in depth.

An attempt has been made to illustrate the board resulting from the practice of this process in Fig. 2, which is double actual size, i. e. the illustration shows a board 1 inch in thickness with an indication of penetration to the extent of  $\frac{1}{8}$  of an inch. Of course it should be taken into consideration that the illustration is more or less diagrammatical, and that there really is no sharp line of demarcation between the de-sized and the sized portions of the board.

It will of course be obvious to those skilled in this art that the mechanical equipment employed may vary considerably from that hereinabove described, and that the main feature to be kept in mind is the application of the aldehyde emulsion or solution to the board at a stage in which it still contains considerable free water.

We claim:

1. Process of producing a size-containing fiber board suitable for the lining of concrete forms, which comprises forming a wet mat from sized lignocellulosic fibers and applying to the still wet surface of said mat on the side intended to contact the wet concrete a composition consisting of a dilute aqueous solution of sodium hydroxide and an aldehyde from the group consisting of formaldehyde and furfural in which the sodium hydroxide is not more than about one-fifth the weight of the aldehyde, and drying the mat.

2. Process of producing a size-containing fiber board suitable for the lining of concrete forms, which comprises forming a wet mat from sized lignocellulosic fibers and applying to the still wet surface of said mat on the side intended to contact the wet concrete a composition consisting of a dilute aqueous solution of sodium hydroxide and formaldehyde, in which the sodium hy-

dioxide is not more than about one-fifth the weight of the formaldehyde and drying the mat.

3. Process of producing a size-containing fiber board suitable for the lining of concrete forms, which comprises forming a wet mat from sized lignocellulosic fibers and applying to the still wet surface of said mat on the side intended to contact the wet concrete a composition consisting of a dilute aqueous solution of sodium hydroxide, furfural and a wetting agent, in which the sodium hydroxide is not more than about one-fifth the weight of the furfural and drying the mat.

4. Process of producing a fiber board suitable for the lining of concrete forms, which comprises forming a wet mat from sized lignocellulosic fibers, and applying to the still wet surface of said mat on the side intended to contact the wet concrete a composition comprising about 20 parts of sodium hydroxide and about 100 parts of furfural dispersed in about 300 parts of water.

5. Process of producing a fiber board suitable for the lining of concrete forms, which comprises forming a wet mat from sized lignocellulosic fibers and applying to the still wet surface of said mat on the side intended to contact the wet concrete a composition comprising about 50 parts of furfural, about 12 parts of sodium hydroxide, and about 8 parts of a wetting agent dispersed in about 300 parts of water.

6. A relatively rigid concrete-form lining material comprising fiber board having its fibers coated with a sizing material throughout the body of the board except on the side intended to contact the wet concrete, on which side the sizing material has been destroyed to a depth of about  $\frac{3}{16}$  of an inch, whereby the said board will be capable of absorbing water from wet concrete in the following proportions: each 16 square inches thereof will absorb between 6 and 16 grams of saturated lime water during the first 15 minutes, 15 to 26 grams in 60 minutes, and 18 to 29 grams in 120 minutes.

7. The concrete-form lining material as defined in claim 6, in which the side of the board in which the sizing material has been destroyed contains fibers carrying an aldehyde.

8. The concrete-form lining material as defined in claim 7 in which the aldehyde is furfural.

9. The concrete-form lining material as defined in claim 7 in which the aldehyde is formaldehyde.

10. Process of rendering a sized wood-fiber board suitable for use as a non-sticking concrete-form material which comprises applying to said board, during a stage in its manufacture where it still contains free moisture, a sufficient amount of an alkaline-reacting emulsion of furfural, containing about one-fifth as much of an alkali as furfural, to desize said board to a depth

of about  $\frac{3}{16}$ " and to leave a film of furfural on the fibers of the board in the desized portions of the latter.

11. The process as defined in claim 10 in which the emulsion is one of furfural in a solution of sodium hydroxide, and there being about five times as much furfural as sodium hydroxide.

12. Process as defined in claim 10 in which the emulsion is one of furfural in a solution of sodium hydroxide also containing a wetting agent not adversely affected by said sodium hydroxide, and there being about five times as much furfural as sodium hydroxide.

13. The process of producing a readily separable concrete form liner which comprises forming a wet mat from conventionally sized lignocellulosic fibers, altering the chemical structure of the fibers and destroying the size thereon in about the surface layer of said wet mat to a depth of about  $\frac{3}{16}$  of an inch by the action of an alkaline reacting solution of an aldehyde from the group consisting of formaldehyde and furfural, and then drying said thus treated mat, the ratio of alkali to aldehyde in said solution being about as 1:5.

ORCUTT W. FROST.  
JAMES H. CONOVER.

#### REFERENCES CITED

30 The following references are of record in the file of this patent:

#### UNITED STATES PATENTS

| Number        | Name             | Date           |
|---------------|------------------|----------------|
| 35 Re. 11,811 | Hall             | Mar. 6, 1900   |
| 52,788        | Gwynn            | Feb. 20, 1866  |
| 1,004,844     | Bennett          | Oct. 3, 1911   |
| 1,637,321     | Johnson          | July 26, 1927  |
| 1,665,236     | Trickey          | Apr. 10, 1928  |
| 40 1,981,405  | Wrede            | Nov. 20, 1934  |
| 1,996,487     | Patrick          | Apr. 2, 1935   |
| 2,010,635     | Kantorowicz      | Aug. 6, 1935   |
| 2,176,981     | Smith et al.     | Oct. 24, 1939  |
| 2,296,553     | Heritage et al.  | Sept. 22, 1942 |
| 45 2,310,400  | Crane et al.     | Feb. 9, 1943   |
| 2,364,772     | Behm             | Dec. 12, 1944  |
| 2,409,629     | Heritage         | Oct. 22, 1946  |
| 2,409,630     | Heritage et al.  | Oct. 22, 1946  |
| 2,432,002     | Frederick et al. | Dec. 2, 1947   |

#### FOREIGN PATENTS

| Number  | Country | Date          |
|---------|---------|---------------|
| 528,030 | Germany | June 24, 1931 |

#### OTHER REFERENCES

55 Paper Industry and Paper World, May 1943, p. 156.

Chemistry of Pulp and Paper Making, Sutermeister, third edition (1941), p. 296 (John Wiley & Sons).